

March 12, 1935.

P. VANET

1,993,812

METHOD FOR PRINTING CINEMATOGRAPHIC FILMS

Filed Jan. 7, 1932



Fig. 1



Fig. 2



Fig. 3

INVENTOR:

Paul Vanet

BY

*Samuel M. Smith*

ATTORNEY

## UNITED STATES PATENT OFFICE

1,993,812

METHOD FOR PRINTING CINEMATO-  
GRAPHIC FILMSPaul Vanet, Le Vesinet, France, assignor to Le  
Film Ozaphane, a corporation of FranceApplication January 7, 1932, Serial No. 585,322  
In France February 16, 1931

3 Claims. (Cl. 95—5)

This invention relates to a method for printing cinematographic films.

There are now to be found in the trade films and photographic papers in which the material sensitive to light comprises a diazo derivative or a stable mixture of a diazo derivative and an azo component.

In the first case, the image is obtained by causing an amine or a phenol in an alkaline medium to act on the film or on the paper after exposure to the sun; in the second case it is sufficient to treat the paper or the film by means of a gaseous alkali or by an alkaline solution after exposure to the sun.

15 The films or papers so prepared yield uninverted images, that is to say a positive is reproduced as a positive and a negative as a negative. It is found, however, that when prints are used which would give correct reproductions on a silver bromide sensitive film, the images obtained on a film which has been sensitized with a diazo compound, show a faulty grading.

20 In order to discover the cause of this abnormal result, I have been led to investigate the manner in which the light acts on the films or papers sensitized by means of diazo derivatives and I have found that the value of the optical densities obtained in function of the amounts of light is governed by a law which widely departs from 25 the law obtained for silver bromide emulsions. It should be remarked, first of all, that said law generally proceeds inversely of the one obtained for bromide, since diazo compounds yield uninverted images.

30 In order to more clearly describe my invention, I have shown several curves in the drawing representing the characteristics of various films.

In the drawing:

Figure 1 shows a set of curves disclosing the comparative results obtained by varied times of exposure.

Fig. 2 shows a curve corresponding to a different density.

Fig. 3 shows a curve corresponding to a still different density.

For the sake of convenience and for a better comprehension of the explanations which will be given hereinafter, I shall trace the characteristic 50 curve representative of the action of light on diazo compounds, plotting as abscissæ the optical densities of a neutral grey corner the densities of which go on increasing from zero, and as ordinates the densities obtained with the diazo compound behind the densities of said neutral

grey corner. The duration of exposure to light will be the same for all parts of the printing.

It is to be noted that this method of constructing the characteristic curve is, in point of fact, just equivalent to the method of Hurter and Driffield, since the axis of the abscissæ figures from right to left lengths which are proportional to the logarithms of the amounts of light transmitted.

10 In treating diazo compound sensitized films, the developments must be carried so far as to develop the whole of the remaining diazo compound, such a protracted development having no effect on the results. Too short a development would leave 15 some diazo compound untransformed into a dye and should always be considered as defective.

If, for a transparent film sensitized with any given diazo compound, I construct the curves corresponding to various and increasing times of exposure  $t_1, t_2, t_3$ , I obtain a sheaf of curves 20  $c_1, c_2, c_3$  such as those shown in Figure 1, which are all similar as to shape but offset with respect to one another. Curve  $c_1$  will correspond to an underexposure, since the high lights of the negative will have a density equal to 1. Curve  $c_2$  will 25 correspond to a correct time of exposure. Curve  $c_3$  will correspond to an overexposure since all the densities of the negative inferior to 0.5 will be rendered by a zero density.

There is, therefore, for this kind of sensitive 30 product, only one correct time of exposure for a negative showing light high lights and half-tints, said time being the one suitable for giving the curve  $c_2$ , and being so determined that it be just sufficient to destroy the whole of the diazo 35 compound behind density 0 of the neutral grey corner or, more precisely, behind the light density corresponding to a high light of the negative. In practice there will be obviously a slight tolerance as to the exact value of this time of exposure.

40 A silver bromide emulsion permits, for a given time of exposure, of obtaining a series of curves the gamma of which varies according to the time of development while a diazo derivative yields but 45 a single curve. Widely different working conditions should, therefore, be expected with the diazo derivative.

As will be apparent, a film sensitized by means 50 of a given amount of diazo compound is characterized firstly by the fact that, on being thoroughly developed without having undergone any exposure to the sun, it will yield a maximum density corresponding to an asymptote which will be horizontal to the characteristic curve. The 55

latter shows a portion which is substantially rectilinear up to a value equal to  $\frac{2}{3}$  or at most to  $\frac{3}{4}$  of the maximum density. If we consider the curve  $c_2$  of Figure 1 which corresponds to 5 a sensitive film adapted to yield a maximum density equal to 2.0 it will be seen that only the portion of the corner having a density increasing from 0 to 1.0 will provide a correct rendering of the densities, the contrast factor excepted, while 10 the rest of the corner is rendered in a defective manner.

In the same way (Figure 2), on the curve corresponding to a density of 3.0 it will be seen that there will be obtained a range of densities correctly increasing from 0 to 2.2 behind the densities of the print increasing from 0 to 1.0, that is to say for illumination values comprised between the value which produces complete discolouring and about one tenth of this value, while 15 beyond there is no longer any proportionateness between the densities of the print and the densities afforded by the diazo compound.

Lastly, a curve such as the one shown by Figure 3 corresponding to a film sensitized by means 25 of a diazo compound in such a way as to provide densities which will exactly reproduce those of the corner between values 0 and 1, that is to say corresponding for this portion to a gamma value equal to unity, will permit of obtaining only a 30 maximum density equal to about 1.4 with an incorrect rendering for all the portions of the print whose density is superior to 1.0. This sort of sensitizing corresponding to the curve shown by Figure 3 is, indeed, the one which has hitherto 35 been prepared by means of diazo compounds.

Now, in cinema practice, it is generally admitted that the image of a positive film properly 40 printed should offer shadows having a maximum density about 2.0 corresponding to the average of good prints the subjects of which, having a variety 45 of luminosity comprised between 1 and 100 or thereabout, are rendered with a product of the gamma of the negative and of the positive equal to unity. Therefore, in order to obtain on a film sensitized by means of a diazo derivative a correct 50 rendering of the images, the following two conditions will have to be performed.

1. To determine for the diazo compound in question the amount to be used for sensitizing the 55 film in such a way as to have a maximum density of about 0.7.

2. To make the positive print which will serve 55 as a matrix with a gamma value sufficiently low in order that the maximum shadow may have a density capable of giving a density equal to 2.0 on the diazo compound.

Practically, in the case contemplated, the value 60 of the maximum density of the positive print, i. e. about 1.0, corresponds to a value of gamma of about 0.5.

Of course, the prints are to be made while using as much as possible the rectilinear portion of the 65 characteristic curve of the silver bromide emulsion and while preferably using an emulsion the characteristic curve of which shows a very long rectilinear portion.

The interest which attaches to my invention resides in the fact that, hitherto, films sensitized by means of diazo compounds were prepared with a low maximum density giving hardly sharp but rather mealy images. As a matter of fact a density of 1.6 was never exceeded, so that the prints used which had themselves a maximum density of about or even above 2.0 with a 75 gamma of about 1. would yield images without

any contrast in the shadows, even when these prints were entirely made on the rectilinear portion of the silver bromide emulsion.

Of course, the use, for printing diazo compound films, of positives having, in the deepest shadows, a maximum density higher than 1.0 but inferior to a limit which may be stated as 1.8, affords an appreciably better general grading of the images and for printing diazo compound sensitized films, I claim the use of positives having a maximum density inferior to 1.8 for a subject the luminosity values of which range from 1 to 100 or thereabout.

Taking the foregoing into account, it becomes obvious that the correlative increase of maximum density which can be afforded by a diazo compound sensitized film already provides a bettering of the grading from a value the minimum of which may be fixed at 1.6.

It is also obvious that the foregoing considerations are particularly applicable to films the images of which show a black or very dark hue, such as a sepia brown or blackish blue, in a word, for colours where sight will readily make, with negligible error, comparative measurements of densities by taking neutral grey as a standard for comparison. Besides, the remarks which have been made will remain applicable, all else remaining equal, when using corners made of a colour identical to the one desired to be compared.

Obviously the conclusions arrived at might 30 be extended to the case where a correct rendering is desired to be effected up to a density value superior to 2.0.

The prints or matrices prepared pursuant to the above set forth principles are practically unsuitable for obtaining proper prints on silver salts, supposing it was desired to use them to prepare counter-types of the prime prints while, on the contrary, on diazo compound sensitive products, they give perfect reproductions.

Such low density matrices for printing diazo compound sensitized films would be useless for projection purposes.

As a practical indication, it is well known that when the gelatine side of a diapositive or transparency giving a good image on projection is applied on very white paper, no detail can be described in the shadows; the image gives the impression of a much overexposed proof on bromide paper, while a matrix prepared according to the conditions set forth in this specification would appear, when applied on white paper, as a bromide proof on paper properly exposed.

Of course, due to the large variety of the diazo compounds suitable for use, it would be impossible to determine in an absolute manner the proportions of diazo compound to be used, otherwise than by indicating that the salt amount should be such as to give an optical density superior to 1.6.

In practice, the method is to be checked as follows:

A sensitizing bath containing the diazo compound having been prepared, the operator will ascertain whether the concentration thereof is proper by dipping thereinto a small fragment of the pellicle to be sensitized and by thoroughly developing the same without any previous exposure to the sun. Then he will measure the density thereof and correct the bath according to the result obtained.

The notion of density as applied to a coloured image may read somewhat ambiguous. It may be made more precise in the following manner.

Supposing a red image projected, for example, by means of a source of light containing red rays and other radiations. The whole of the red rays passes through all the parts of the print. There will then be considered as a density equal to unity an intensity of the red colouring such that  $\frac{1}{6}$  of the rays other than the red ones (in the case in point) are absorbed, so that the light transmitted is only  $\frac{1}{6}$  of the incident light for those rays.

The conclusions that are the object of this specification apply in the same conditions and by observing the same proportions to photographic papers which are based on the use of diazo derivatives and prepared especially in view of reproducing not line engraving but process plates.

I claim:

1. In a method of preparing diazo compound sensitized films, comprising applying sufficient diazo compound sensitized material to the film to give a maximum optical density above 1.6, the steps of using as matrices for printing the films, natural or toned silver salt prints or films developed with a gamma sufficiently low in order that the darkest shadow be rendered on the diazo compound sensitized film by a density lower than  $\frac{3}{4}$  of the maximum density which would be pro-

vided without any exposure to light by said diazo compound sensitized film.

2. In a method of preparing diazo compound sensitized films, comprising applying sufficient diazo derivatives to a regenerated cellulose film to give a maximum optical density above 1.6, the steps of using as matrices for printing the films, natural or toned silver salt prints or films developed with a gamma sufficiently low in order that the darkest shadow be rendered on the diazo compound sensitized film by a density lower than  $\frac{3}{4}$  of the maximum density which would be provided without any exposure to light by said diazo compound sensitized film.

3. In a method of preparing films sensitized with diazo compounds applied on a support of regenerated cellulose, the steps of using for printing, positive matrices of silver salts, black or toned and developed with a gamma sufficiently low in order that the darkest shadows be rendered on the sensitive film with a density lower than  $\frac{3}{4}$  of the maximum density which would be provided without any exposure of the diazo compound sensitized film to light, the concentration of the film in diazo compound being fixed so that the gradation of the images obtained on the film will be normal for the projection.

PAUL VANET.